

## 1

3,529,654

### IMPROVING THE SURFACE OF FERROUS ARTICLES BY COMPLEXING AGENTS

Jerome J. Kanter, Palos Park, Ill., assignor to Crane Co., Chicago, Ill., a corporation of Illinois  
No Drawing. Filed Feb. 15, 1968, Ser. No. 705,614  
Int. Cl. B22c 3/00; B22d 27/18  
U.S. Cl. 164—58

3 Claims

#### ABSTRACT OF THE DISCLOSURE

A process for forming a hard, durable, corrosion resistant coating on a cast ferrous article by applying a wash comprising an aqueous solution of sodium chromate, sodium aluminate, aluminum hydrate, or the rare earth metal hydrates to the surface of a mold cavity. During casting, a mineral oxide complex of the spinel type is formed on the surface of the cast ferrous article.

#### BACKGROUND OF THE INVENTION

An article fabricated of ferrous metal has a strong propensity to corrode unless the metal is extensively alloyed with a non-ferrous metal such as chromium, for example, or the article is provided with a protective coating. A cast or wrought iron, as well as a plain carbon steel, will readily corrode in an atmosphere where oxygen is present unless a protective coating is formed on the surface of the article. Since the use of a "stainless" steel, for example, in numerous applications where requirements dictate fabrication of an article in iron or steel, is prohibitively expensive, numerous coating and other surface protection methods have been developed.

The most commonly used simple coating for metal articles is paint. Another coating widely used on ferrous metal articles is zinc; i.e. galvanizing. Chrome plating is also employed where a hard and attractive surface is desirable.

Each of the aforementioned methods necessarily requires performing a separate step after fabrication of the articles. This adds to production costs. Where a metallic coating such as chromium, for example, is applied, the increased cost factor is substantial. On the other hand, whereas a paint coating is considerably less expensive, it is also unsuitable in numerous applications of the ferrous article because the article is employed in an environment where the paint itself is attacked and readily breached.

In contrast to the known processes where a protective coating is provided after the metal article is fabricated, methods have been developed for forming an alloy-type coating on the cast metal during the casting operation. A process of this nature is described in U.S. Pat. No. 1,725,039, where a chromium alloy surface is formed on a ferrous article by coating the mold surface with a chromium powder and an oxide formation inhibitor in an organic binder. The metallic chromium alloys with the molten base metal at the surface of the cast article.

In a broadly similar process, a hard surface coating of tungsten or molybdenum carbide is formed on a cast base metal by painting the mold cavity with the finely powdered coating material in a binder. The carbide coating formed on the surface of the base metal is highly resistant to wear and certain types of corrosion. This process is disclosed in U.S. Pat. No. 1,981,403.

These two surface coating processes offer distinct advantages in the formation of protective surfaces on base metal castings in that the protective coatings are formed during the casting operation. There are other coating or surface treatment processes of this general nature, of course. None provides the ultimate simplicity and mini-

## 2

mum cost factors which are highly desirable and constantly sought, however.

#### SUMMARY OF THE INVENTION

The present invention is directed to an improved process for forming a hard, durable, corrosion resistant coating on ferrous articles. More particularly, it relates to the development of a corrosion resistant surface on cast ferrous articles. It is an object of the invention to provide a process for forming an extremely hard, durable, corrosion resistant coating on a cast ferrous article by a simple and inexpensive treatment of the mold prior to casting the article. A further object of the invention is to provide a process wherein painting a mold cavity with a wash containing one or more compounds of a group consisting of sodium chromate, sodium aluminate, aluminum hydrate, and the rare earth metal hydrates, prior to casting, results in a mineral oxide complex of the spinel type being formed on the surface of the cast ferrous metal articles.

To the accomplishment of the foregoing related ends, the invention comprises the features hereinafter clearly described and pointed out in the claims, the following description setting forth in detail certain illustrative embodiments of the invention. It should be understood, however, that these are indicative of but a few of the various ways in which the principles of the invention may be employed.

#### DESCRIPTION OF THE PREFERRED EMBODIMENTS

Briefly stated, the present invention contemplates painting or daubing a wash containing a compound from a group consisting of sodium chromate, sodium aluminate, aluminum hydrate, and the rare earth metal hydrates, on the cavity surface in a mold. The cavity might be formed in a green sand mold or a chill mold, for example. The mold might be baked to a dry sand mold subsequent to the wash being applied or the wash might be applied directly to a dry sand mold.

A molten ferrous base metal is introduced to the treated (painted or daubed) mold cavity. As the base metal solidifies in the cavity, the presence of free oxygen at the interface between the article and the mold causes oxidation to take place. Without prior treatment of the mold according to the invention, this oxidation would normally result in the formation of the base metal oxide on the article surface.

The normally formed base metal oxide would, of course, offer some resistance to corrosion. However, it is not a hard, durable surface which is highly resistant to corrosion in high temperature and pressure environments.

In the present invention, a more complex oxide is formed from both the base metal and the metallic element(s) in the compound(s) washed onto the surface of the mold cavity prior to casting. The complex oxide is of the spinel type. In this light, the spinels are generally defined as a group of isomorphous mineral oxides having the generic formula  $AB_2O_4$  where A is ferrous iron, and B is one of a group of minerals including aluminum, chromium, and the rare earth elements.

A spinel type oxide complex is characterized by its gem-like hardness. It constitutes a durable and extremely corrosion resistant coating on the base metal. The coating, because of its hardness and durability, is highly corrosion resistant under extremely adverse conditions, including those aforementioned conditions where high temperatures and pressures are encountered and corrosion is normally a serious problem.

The use and application of the process embodying features of the invention may best be understood by reciting an example. A boiler casting is necessarily exposed to the corrosive and erosive action of fluids under high pressures

and temperatures on its inner surfaces. Because of the economic factors involved in providing a corrosion resistant coating on the exposed inner surface of such a casting by conventional and well-known techniques, it is customary in boiler castings to rely on the oxide coating normally formed on the surface during casting as a corrosion inhibitor. Unfortunately, although this oxide coating does provide a certain deterrent factor, corrosion still occurs at a rapid rate because of the nature of the environment.

To make the inner surface of the boiler casting highly corrosion resistant according to the present invention, a wash is prepared comprising a solution of sodium chromate ( $Na_2CrO_4$ ), for example, in water. At the same time, a conventional green sand mold, for example, is prepared. The wash is painted or daubed on the surface of the mold cavity where a corrosion resistant surface is desired on the article being cast. The green sand mold is then baked at approximately  $400^{\circ} F.$ – $600^{\circ} F.$  to form a dry sand mold with the sodium chromate present on the mold cavity surfaces which have been treated with the wash.

The mold having been prepared in the aforescribed manner, molten ferrous iron is introduced to the mold cavity by conventional techniques. The molten iron solidifies in the mold to form the article being cast; in the present instance, a boiler casting. The normal presence of oxygen in the sand at the interface between the solidifying article and the mold surface causes oxidation of the casting base metal to take place on the casing surface.

In the present invention this oxidation process is more complex than merely a formation of base metal oxide. As the ferrous iron oxidizes, the chromium in the sodium chromate is taken into the oxidation reaction. A new and complex oxide of the spinel type is formed on the surface of the article by the oxidation process. In the present example, this compound comprises iron chromium oxide or  $FeCr_2O_4$ .

The spinel-like oxide complex which forms on the surface of the cast ferrous article has, in a characteristic manner, a gem-like hard surface. This surface is extremely durable and corrosion resistant under the substantially adverse conditions to which a boiler casting inner surface is subjected; i.e. high pressures and temperatures.

In the example utilized, the "mold" has been described as a green sand mold which is baked to a dry sand mold prior to casting and after the "wash" is applied. It should be reiterated here that the invention also contemplates applying the wash to a chill mold, for example, or a dry sand mold *after* baking. It is further within the purview of the invention that the wash be applied and the invention employed with various other types of molds.

In addition, the exemplary wash employed is an aqueous solution of sodium chromate. The wash might, however, comprise a sodium aluminate, aluminum hydrate, or rare earth metal hydrate compound in an aqueous solution. In any such case a hard, durable, corrosion resistant surface of the nature contemplated is formed.

In this light, although the resultant hard, durable, corrosion resistant surface which forms on the ferrous metal casting according to the invention has been described as a

spinel-type oxide complex, it is possible that the hard coating might comprise other elements or more or less complex compounds. Such an eventuality and resultant surface coating make-up are also within the contemplation of the invention.

Regardless, the corrosion resistant surface which is formed on the surface of a cast metal article such as a boiler casting or the like by the process embodying features of the invention is highly effective under the most adverse conditions. Nevertheless, the process itself is exceedingly simple and inexpensive. Cast ferrous articles can be made with highly corrosion resistant surfaces at costs compatible with their applications.

While the embodiment described herein is at present considered to be preferred, it is understood that various modifications and improvements may be made therein, and it is intended to cover in the appended claims all such modifications and improvements as fall within the true spirit and scope of the invention.

What is desired to be claimed and secured by Letters Patent of the United States is:

1. A process for forming a protective coating on a cast ferrous article comprising the steps of:

- (a) treating a surface of a mold cavity with a compound or compounds from a group consisting of sodium aluminate, sodium chromate, aluminum hydrate, and the rare earth metal hydrates,
- (b) and introducing molten ferrous metal to the cavity so that it forms a casting which comes into contact with said compound at said surface,
- (c) whereby a chemical complex coating is formed on the casting and said complex coating has a hard, corrosion resistant surface.

2. The process of claim 1 further characterized in that:

- (a) said compound is coated on said mold cavity by applying a liquid wash containing the compound to the walls of the cavity.

3. The process of claim 1 further characterized in that:

- (a) said mold cavity is formed in a green sand mold,
- (b) said mold cavity is coated with said compound by preparing a liquid wash containing said compound and coating the cavity with said wash,
- (c) said green sand mold being baked for a predetermined length of time after the application of said wash and before introducing the molten ferrous metal to the cavity to form a dry sand mold.

#### References Cited

##### UNITED STATES PATENTS

|           |          |              |       |        |
|-----------|----------|--------------|-------|--------|
| 1,166,167 | '12/1915 | Woods        | ----- | 164—58 |
| 2,847,741 | 8/1958   | Meves et al. | ----- | 164—14 |
| 3,121,269 | 2/1964   | Neff         | ----- | 164—14 |

55 J. SPENCER OVERHOLSER, Primary Examiner

J. E. ROETHEL, Assistant Examiner

#### U.S. CL. X.R.

106—38.27; 117—5.2; 164—14, 72, 138